



US005308472A

**United States Patent** [19]

Dai et al.

**[11] Patent Number:** 5,308,472  
**[45] Date of Patent:** May 3, 1994

[54] **MILD HYDROCRACKING PROCESS USING CATALYSTS CONTAINING DEALUMINATED Y-ZEOLITES**

[75] Inventors: **Pei-Shing E. Dai; Charles N. Campbell, II, both of Port Arthur; Bobby R. Martin; David E. Sherwood, Jr., both of Beaumont, all of Tex.**

[73] Assignee: **Texaco Inc.**, White Plains, N.Y.

[21] Appl. No.: **897,167**

[22] Filed: **Jun. 11, 1992**

[51] Int. Cl.<sup>5</sup> ..... **C10G 47/14**

[52] U.S. Cl. ..... **208/111; 208/216 PP;**  
..... **208/251 H**

[58] Field of Search ..... **208/111, 216 PP**

[56] **References Cited**

**U.S. PATENT DOCUMENTS**

|           |         |                |         |
|-----------|---------|----------------|---------|
| 4,430,200 | 2/1984  | Shihabi        | 208/120 |
| 4,533,533 | 8/1985  | Dewing et al.  | 423/328 |
| 4,600,498 | 7/1986  | Ward           | 208/111 |
| 4,654,454 | 3/1987  | Barri et al.   | 585/415 |
| 4,738,766 | 4/1988  | Fischer et al. | 208/111 |
| 4,789,457 | 12/1988 | Fischer et al. | 208/111 |
| 4,826,587 | 5/1989  | Ward et al.    | 208/111 |
| 4,857,169 | 8/1989  | Abdo           | 208/111 |
| 4,869,803 | 9/1989  | Ward           | 208/111 |
| 4,879,019 | 11/1989 | Ward           | 208/111 |
| 4,894,142 | 1/1990  | Steigleder     | 208/111 |

|           |         |                |         |
|-----------|---------|----------------|---------|
| 4,919,787 | 4/1990  | Chester et al. | 208/52  |
| 4,923,592 | 5/1990  | Abdo           | 208/111 |
| 4,960,505 | 10/1990 | Minderhoud     | 208/111 |
| 5,037,531 | 8/1991  | Budens et al.  | 208/120 |
| 5,053,374 | 10/1991 | Absil et al.   | 502/64  |
| 5,069,890 | 12/1991 | Dai et al.     | 423/328 |
| 5,087,348 | 2/1992  | Dai et al.     | 208/111 |
| 5,112,473 | 5/1992  | Dai et al.     | 208/111 |

*Primary Examiner*—Helane Myers

*Attorney, Agent, or Firm*—James L. Bailey; Kenneth R. Priem; Walter D. Hunter

[57]

**ABSTRACT**

A mild hydrocracking process for the hydrodemetallation (HDM), hydrodesulfurization (HDS) and hydroconversion (HC) of hydrocarbon feedstocks such as residuum feedstocks which provides increased conversion of heavy hydrocarbons boiling above 1000° F. into products boiling below 1000° F. as well as increased yields of middle distillates is disclosed. The process utilizes a catalyst comprising about 1.0 to about 6.0 wt. % of an oxide of a Group VIII metal, about 12.0 to about 25.0 wt. % of an oxide of molybdenum and 0.1 to about 5.0 wt. % of an oxide of phosphorus supported on a porous support comprising precipitated alumina or silica-containing alumina and hydrogen form, acidified, dealuminated Y-zeolite.

6 Claims, No Drawings

MILD HYDROCRACKING PROCESS USING  
CATALYSTS CONTAINING DEALUMINATED  
Y-ZEOLITES

BACKGROUND OF THE INVENTION

1. Field of the Invention

This invention relates to a catalytic process for mild hydrocracking of heavy oils. More particularly, this invention relates to a mild hydrocracking process for the hydrodemetallation (HDM), hydrodesulfurization (HDS) and hydroconversion (HC) of a heavy hydrocarbon feedstock boiling above 650° F., such as vacuum gas oil (VGO) and VGO containing a high proportion of vacuum resid (VR) to lighter distillate products boiling at or below 650° F.

In the mild hydrocracking process of this invention a sulfur- and metal-containing hydrocarbon feedstock, such as residue containing heavy oils, is contacted at an elevated temperature with hydrogen and a catalyst composition comprising a specified amount of a Group VIII metal, such as an oxide of nickel or cobalt, a specified amount of an oxide of molybdenum and, optionally, a specified amount of an oxide of phosphorus, such as phosphorus pentoxide supported on a porous alumina support containing a dealuminated Y-zeolite. In the catalytic mild hydrocracking process of this invention the sulfur- and metal-containing hydrocarbon feed is contacted with hydrogen and the catalyst containing a hydrogen form, acidified, dealuminated Y-zeolite, which has a specified pore size distribution, in a manner such that an increased production of middle distillates and a substantially higher conversion of the 1000° F. + fraction of the hydrocarbon feed to the 1000° F. - lighter products is achieved over that obtained with the use of prior art hydroprocessing catalysts while high levels of sediment formation are avoided.

2. Prior Art

U.S. Pat. No. 4,600,498 (Ward) teaches a process for mild hydrocracking a hydrocarbon oil having a substantial proportion of components boiling below about 1100° F. which comprises contacting the hydrocarbon oil under conditions of elevated temperature and a hydrogen pressure less than about 1500 psig with a particulate catalyst comprising at least one hydrogenation component, a Y-zeolite having a unit cell size between about 24.40 and 24.64 Å and a dispersion of silica-alumina in a matrix consisting essentially of alumina.

U.S. Pat. No. 4,894,142 (Steigleider) discloses a highly selective hydrocracking process providing increased yields of middle distillates. The process employs a catalyst comprising a hydrogen form Y-type zeolite having a unit cell size between about 24.20 Angstroms and 24.40 Angstroms, a metal hydrogenation component and refractory oxide support materials. The catalyst is characterized by low ammonia temperature programmed desorption (TPD) acidity strength which may be achieved by dehydroxylation caused by a dry calcination.

U.S. Pat. No. 4,430,200 (Shihabi) discloses hydrocarbon conversion catalysts having reduced aging rates and exhibiting lower gas yield in conversion processes made by presteaming a large pore, high silica zeolite such as mordenite or zeolite Y and base-exchanging the steamed zeolite with an alkali metal to reduce the acidity to a low value.

U.S. Pat. No. 4,654,454 (Barri, et al.) discloses a process for converting C<sub>2</sub> to C<sub>5</sub> hydrocarbons to aromatic

hydrocarbons which comprises bringing the hydrocarbon into contact with a surface dealuminated zeolite loaded with a gallium compound.

U.S. Pat. No. 4,533,533 (Dewing, et al.) discloses a process for selective and controlled dealumination of an alumino silicate zeolite by heating a zeolite having pores filled with coke in air at a temperature of 450° C.-650° C. The partially dealuminated zeolite is useful in toluene disproportionation processes.

U.S. Pat. No. 5,069,890 (Dai, et al.) discloses novel treated zeolite, such as Y-zeolite, prepared by treating charge zeolite, such as a dealuminated Y-zeolite (which is essentially free of Secondary Pores), with steam for 5-60 hours at 1000° F.-1500° F. Product is particularly characterized by increased Secondary Pore Volume (pores of diameter of 100A-600A) in amount of as high as 0.20 cc/g and is useful in resid hydroprocessing.

U.S. Pat. No. 5,053,374 (Absil, et al.) discloses low acidity refractory oxide-bound zeolite catalysts, for example, silica-bound ultrastable Y-zeolite, possessing physical properties, e.g., crush strength similar to those of their alumina-bound counterparts, and since low acidity refractory oxide-bound catalysts are inherently less active than alumina-bound zeolite catalysts, the former are particularly useful in hydrocarbon conversion processes in which reduced coke make increased catalyst cycle length. Due to their stability in acid environments, the low acidity refractory oxide-bound zeolite extrudate can be acid treated without unduly compromising structural integrity.

U.S. Pat. No. 4,919,787 (Chester, et al.) discloses an improved method for passivating metals in a hydrocarbon feedstock during catalytic cracking which involves contacting the feedstock with a passivating agent comprising a precipitated porous rare earth oxide, alumina, and aluminum phosphate precipitate. The passivating agent may be coated on a cracking catalyst, such as dealuminated Y-zeolite, Y-zeolite, etc., be part of the matrix of a cracking catalyst, or be added to the cracking operations as discrete particles.

U.S. Pat. No. 5,037,531 (Bundens, et al.) discloses a catalytic cracking process using a catalyst comprising a framework dealuminate Y-zeolite which is rare earth and aluminum exchanged.

SUMMARY OF THE INVENTION

The instant invention is a process of mild hydrocracking of a sulfur- and metal-containing hydrocarbon feedstock having a substantial proportion of components boiling below about 1000° F., such as residue, vacuum gas oils, etc., which comprises contacting the feedstock at an elevated temperature and at a pressure of less than 1500 psig with hydrogen and a catalyst which comprises about 1.0 to about 6.0 wt. %, preferably about 2.5 to about 3.5 wt. % of an oxide of a Group VIII metal, preferably nickel or cobalt; about 12.0 to about 25.0 wt. %, preferably about 12.0 to about 18.0 wt. % of an oxide of molybdenum; about 0 to about 5.0 wt. %, preferably about 0 to about 2.0 wt. % of an oxide of phosphorus, preferably P<sub>2</sub>O<sub>5</sub>, all supported on a porous support comprising (1) a matrix selected from the group consisting of precipitated alumina and silica-alumina containing about 1.0 to about 3.0 wt. % silica, and (2) about 5.0 to about 35.0 wt. %, based on the weight of the support, of a hydrogen form, acidified, dealuminated Y-zeolite having a unit cell size of less than about 24.35 Angstroms, preferably about 24.15 to about 24.35

Angstroms. The catalyst is characterized by having a total surface area of about 200 to about 300 m<sup>2</sup>/g and a total pore volume of about 0.55 to about 0.75 cc/g, preferably about 0.60 to about 0.70 cc/g, with a pore volume distribution such that micropores having diameters less than 100 Å constitute less than 40%, pores having diameters of 100-160 Å constitute about 25 to about 50%, pores having diameters greater than 160 Å constitute about 25 to about 50%, of the total pore volume of the catalyst and, macropores having diameters greater than 250 Å constitute about 15 to about 40% preferably about 18 to about 35%, and macropores having diameters greater than 1500 Å constitute less than 10% of the total pore volume. The catalyst is further characterized by having about 40 to about 65% of the total pore volume in pores of diameters from about 20 Å below the pore mode diameter to about 20 Å above the pore mode diameter, and the pore mode diameter is in the range of about 80 to about 120 Angstroms.

The hydrogen form, acidified, dealuminated Y-zeolite employed in preparing the catalyst support is further characterized by having the total pore volume of secondary pores of diameter greater than 100 Å of at least 0.13 cc/g, which correspond to 45% of total pore volume and the pore mode of the secondary pores is in the range of 115-145 Å. The catalyst support has a modified monomodal pore size distribution optimized for reducing the sediment make.

This invention also relates to the catalyst employed in the described process. The molybdenum gradient of the catalyst ranges from about 1 to about 20, preferably from about 1.0 to about 5.0.

The operating conditions for the process of the instant invention are such as to yield about a 10 to about 30 vol. % conversion of the hydrocarbon feedstock boiling at 650° F. + to hydrocarbon products boiling at 650° F. -.

The residuum feedstocks may be contacted with hydrogen and the catalyst utilizing a wide variety of reactor types. Preferred means for achieving such contact include contacting the feed with hydrogen and the prescribed catalyst in a fixed bed hydrotreater, in a single continuous-stirred-tank reactor or single ebullated-bed reactor, or in a series of 2-5 continuous-stirred-tank or ebullated-bed reactors, with ebullated-bed reactors being particularly preferred. The process of the instant invention is particularly effective in achieving high conversion rates with increased production of middle distillate and 1000° F. - fractions having the desired degree of hydrodesulfurization (HDS) while at the same time the sediment make is maintained at a level similar to that resulting from the use of conventional bimodal alumina-based catalysts.

#### DESCRIPTION OF THE PREFERRED EMBODIMENTS

The decreasing demand for heavy fuel oils has caused refiners to seek ways to convert heavier hydrocarbon feedstocks to lighter products of more value. To increase mid-distillate production as well as to increase the conversion of the 100° F. + fraction to the 1000° F. - fraction, the refiner has several process options. They include hydrocracking, fluid catalytic cracking, and coking, which all require heavy investments in the refineries. Because of such high costs, refiners are continually searching for conversion processes which may be utilized in existing units. An additional option avail-

able to refiners is to employ a mild hydrocracking (MHC) process. MHC is process is an evolution of the VGO hydrodesulfurization (HDS) process. The main feedstock for this MHC process is VGO but other types of heavy gas oils, such as coker gas oils and deasphalted oils, can be used.

The major advantage of MHC is that it can be carried out within the operating constraints of existing VGO hydrotreaters. The typical conditions for the MHC process are: Temperature: 720°-780° F., Hydrogen Pressure: 600-1200 psig, H<sub>2</sub>/Oil Ratio: 1000-2000 SCF/BBL, Space Velocity: 0.4-1.5 Vol/Vol/Hr. In contrast, true high conversion hydrocracking units are operated at these conditions: Temperature: 700°-900° F., Hydrogen Pressure: 1800-3000 psig, H<sub>2</sub>/Oil Ratio: 1400-8000 SCF/BBL, Space Velocity: 0.3-1.5 Vol/Vol/Hr. The major difference between the two processes is the hydrogen pressure.

The products obtained from the MHC process are low sulfur fuel oil (60-80%) and middle distillate (20-40%). This hydrotreated fuel oil is also an excellent feed for catalytic cracking because of its higher hydrogen content and lower nitrogen content compared to the original feed. The quality of diesel cut produced by MHC is usually close to diesel oil in specifications for the cetane index, and so can be added to the diesel pool.

The switch from a HDS mode to a MHC mode can be achieved in different ways, assuming that the refiner is equipped to recover the surplus of the middle distillate fraction. One way to increase middle distillate production from a unit loaded with HDS catalyst is to increase the operating temperature. Using a conventional hydrotreating catalyst, the MHC process typically converts about 10 to 30 Vol. % of hydrocarbon feedstock boiling above 650° F. (650° F. +) to middle distillate oils boiling at or below 650° F. (650° F. -).

Another way to increase the middle distillate production is to change, at least partly, a HDS catalyst on a nonacidic alumina support to a slightly acidic catalyst. Catalysts of higher hydrogenation activity and/or hydrocracking activity are still being sought. The higher the hydrogenation activity of the catalyst, the lower the temperature required to obtain a product of given sulfur, nitrogen or metal content in any given boiling range. For the VGO containing a high proportion of residuum, an HDS catalyst usually gives less than 10 Vol. % conversion of the 650° F. - fraction. The conversion of resid components boiling above 1000° F. (1000° F. +) into products boiling at or below 1000° F. (1000° F. -) with the known alumina-based hydrotreating catalysts is achieved primarily by thermal cracking reactions.

A particular difficulty which arises in resid hydroprocessing units employing the currently known catalysts is the formation of insoluble carbonaceous substances (also called sediment) when the conversion is high (above 50 Vol. %). High sediment may cause plugging of reactor or downstream units, such as a fractionation unit. The higher the conversion level for a given feedstock, the greater the amount of sediment formed. This problem is more acute at a low hydrogen pressure and high reaction temperature.

The process of the instant invention employs a catalyst composition comprising about 1.0-6.0, preferably 2.5-3.5 wt. % of an oxide of a Group VIII metal, preferably nickel or cobalt, most preferably NiO, about 12.0 to about 25.0 wt. %, preferably about 12.0 to about 18.0 wt. % of an oxide of molybdenum, about 0 to about 5.0

wt. %, preferably 0.1 to about 2.0% of an oxide of phosphorus, preferably  $P_2O_5$ , all supported on a support comprising (1) a matrix selected from the group consisting of precipitated alumina and alumina containing about 1.0 to about 3.0 wt. % silica, and (2) about 5.0 to about 35 wt. %, based on the weight of the support, of a hydrogen form, acidified, dealuminated Y-zeolite having a unit cell size of less than 24.35 Å and preferably about 24.15 to about 24.35 Å.

As previously mentioned, the catalyst is further characterized by having a total surface area of about 200 to about 300  $m^2/g$  and a total pore volume of about 0.55 to about 0.75 cc/g, preferably about 0.60 to about 0.70 cc/g with a pore volume distribution such that micropores having diameters less than 100 Å constitute less than 40%, pores having diameters of 100-160 Å constitute about 25 to about 50%, pores having diameters greater than 160 Å constitute about 25 to about 50%, of the total pore volume of the catalyst, macropores having diameters greater than 250 Å constitute about 15 to about 40%, preferably about 18 to about 35%, and macropores having diameters greater than 1500 Å constitute less than 10% of the total pore volume. Pore diameters were measured using a Micromeritic instrument, Autopore 9220 V 2.03.

The catalyst is also further characterized by having about 40 to about 65% of the total pore volume in pores of diameters from about 20 Angstroms below the pore mode diameter to about 20 Å above the pore mode diameter and the pore mode diameter is in the range of about 80 to about 120 Å.

The hydrogen form, acidified, dealuminated Y-zeolite utilized in preparing the catalyst support is further characterized by having the total pore volume of secondary pores of diameters greater than 100 Angstroms is at least 0.13 cc/g which corresponds to 45% of the total pore volume and the pore mode of the secondary pores is in the range of 115-190 Angstroms.

Group VIII, as referred to herein, is Group VIII of the Periodic Table of Elements. The Periodic Table of Elements referred to herein is found on the inside cover of the CRC *Handbook of Chemistry and Physics*, 55th Ed. (1974-75). Other oxide compounds which may be present include  $SO_4$  (present in less than 0.8 wt. %), and  $Na_2O$  (present in less than 0.1 wt. %). The above-described support may be purchased or prepared by methods well known to those skilled in the art.

The hydrogen form, acidified, dealuminated Y-zeolites employed in preparing the catalysts of this invention may be characterized by various properties such as pore size, unit cell size, silica to alumina mole ratio, pore mode, etc.

**Primary Pore Size**—The primary pores are small pores characterized by a pore diameter of less than about 100 Angstroms. Such small or micropores are commonly present together with super micropores having a pore diameter of 40-100 Angstroms. Pore size is measured by nitrogen desorption isotherm.

**Primary Pore Volume**—The volume of the primary pores.

**Primary Pore Mode**—The pore diameter of pores where a maximum occurs in the pore volume distribution curve within the range of pore diameters of 20-100 Å.

**Unit Cell Size**—The unit cell size or lattice content is measured by X-ray diffraction.

**Secondary Pore Size**—The secondary pores are large pores characterized by a pore diameter of greater than

100 Angstroms, typically 100-600 Angstroms. The pore size is measured by nitrogen desorption isotherm.

**Secondary Pore Volume**—The hydrogen form acidified dealuminated Y-zeolites employed in the catalysts of this invention are characterized by having a secondary pore volume as measured by nitrogen desorption isotherm.

**Secondary Pore Mode**—The pore diameter of pores where a maximum occurs in the pore volume distribution curve within the range of pore diameters of 100-600 Å.

Hydrogen form dealuminated Y-zeolites useful in preparing the hydrogen form, acidified, dealuminated Y-zeolite previously described include, for example:

A. The Valfor CP 300-35 grand of super ultrastable Y-zeolite of PQ Corp.

B. The Valfor CP 304-37 brand of super ultrastable Y-zeolite of PQ Corp.

The properties of zeolites A and B are set out in Table 1 which follows.

TABLE I

| Property                   | ZEOLITE |       |
|----------------------------|---------|-------|
|                            | A       | B     |
| Primary Pore Size Å        | 85      | 39    |
| Primary Pore Volume cc/g   | 0.11    | 0.11  |
| Lattice Constant           | 24.35   | 24.37 |
| Secondary Pore Size (Å)    | none    | 115   |
| Secondary Volume cc/g      | 0.12    | 0.12  |
| Total Pore Volume cc/g     | 0.23    | 0.23  |
| Total Surface Area $m^2/g$ | 580     | 620   |
| Crystallinity %            | 87      | 74    |
| $SiO_2$ to $Al_2O_3$       |         |       |
| Mole Ratio (XRD)           | 18      | 16    |
| Acid Site Density cc/g     | 6.5     | 13    |

The preferred zeolite is a zeolite such as the CP-300-35 brand of Y-type zeolite of PQ Corp.

Dealuminated Y-zeolites useful in preparing the hydroprocessing catalysts of this invention include hydrogen form, acidified, dealuminated Y-zeolites having a silica to alumina mole ratio of about 10-120 characterized by (a) secondary pore volume of about 0.14-0.20 cc/g, (b) a unit cell size of about 24.23-24.33 Å, (c) a secondary pore mode of about 115-145 Å, (d) a secondary pore diameter of about 100-600 Å, (e) a surface silicon to aluminum atom ratio of about 24-45, and (f) an acid site density of about 1-5 cc  $NH_3/g$  of zeolite.

The acidified, dealuminated Y-zeolites suitable for use in forming the hydroprocessing catalysts of this invention are prepared by contacting the hydrogen form of a dealuminated Y-zeolite having a silica to alumina mole ratio of about 10-120 and a unit cell size of about 24.30-24.50 Å at a temperature of 75°-140° F. for 0.5-6 hours with an acidic medium, such as an aqueous solution of an organic acid, such as citric or acetic acid, or an aqueous solution of an inorganic acid, e.g., nitric acid or hydrochloric acid; thereby converting the starting dealuminated Y-zeolite into an acidified zeolite characterized by (a) an increased secondary pore volume of about 0.14-0.20 cc/g, (b) a decreased unit cell size of about 24.23-24.33 Å, (c) a secondary pore mode of about 115-145 Å, (d) a secondary pore diameter of about 100-600 Å, and (e) a surface silicon to aluminum atom ratio of about 24-45.

In preparing the hydrogen form acidified, dealuminated Y-zeolite, which can be employed in making the catalyst composition of this invention, a charge zeolite, such as Valfor CP-300-35 USY, for example (as crystals of particle size of 0.2-0.4 microns), is contacted with

0.5N aqueous nitric acid (5000 parts per 100 parts of zeolite) at 140° F. for 2 hours. The aqueous liquid is then removed and the acidified zeolite product dried for 24 hours at 250° F. The properties of the hydrogen form, acidified, dealuminated Y-zeolite product and the properties of the charge zeolite are set out in Table II which follows.

TABLE II

| Property                                                     | Charge Zeolite | Acidified Zeolite |
|--------------------------------------------------------------|----------------|-------------------|
| Primary Pore Mode A                                          | 85             | 43                |
| Primary Pore Volume, cc/g                                    | 0.11           | 0.11              |
| Unit Cell Size A                                             | 24.35          | 24.25             |
| Secondary Pore Volume, cc/g                                  | 0.12           | 0.17              |
| Secondary Pore Mode A                                        | 0              | 135               |
| Total pore Volume, cc/g                                      | 0.23           | 0.28              |
| Total Surface Area, m <sup>2</sup> /g                        | 580            | 730               |
| Crystallinity %                                              | 87             | 94                |
| SiO <sub>2</sub> :Al <sub>2</sub> O <sub>3</sub> Ratio (XRD) | 18             | 54                |
| Acid Site Density                                            | 6.5            | 2.9               |
| cc NH <sub>3</sub> /g                                        | 1.6            | 24                |
| Surface Si:Al Ratio                                          |                |                   |

The preparation of the hydrogen form, acidified, dealuminated Y-zeolites is more completely described in U.S. patent application Ser. No. 07/533,222 filed Jun. 4, 1990, now U.S. Pat. No. 5,112,473, which is incorporated herein by reference in its entirety.

#### Catalyst Preparation

In preparing the catalyst the above-described support is impregnated with the requisite amounts of molybdenum oxide, Group VIII metal oxide and phosphorus oxide via conventional means known to those skilled in the art to yield a finished catalyst containing a Group VIII metal oxide in the amount of 1.0 to about 6.0 wt. %, preferably about 2.5 to about 3.5 wt. %, is molybdenum oxide in the amount of 12.0 to about 25.0 wt. %, preferably 12.0 to about 18.0 wt. % and phosphorus oxide in the amount of about 0 to about 5.0 wt. %, preferably 0 to about 2.0 wt. %.

The Group VIII metal may be iron, cobalt or nickel which is loaded on the support, for example, as a 10-30 wt. %, preferably about 15 wt. % of an aqueous solution of metal nitrate. The preferred metal of this group is nickel which may be employed at about 16 wt. % aqueous solution of nickel nitrate hexahydrate. Molybdenum may be loaded on the support employing, for example, a 10-20 wt. %, preferably about 15 wt. %, of an aqueous solution of ammonium heptamolybdate (AHM). The phosphorus component may be derived from 85% phosphoric acid.

The active metals and phosphorus may be loaded onto the catalyst support via pore filling. Although it is possible to load each metal separately, it is preferred to

impregnate simultaneously with the Group VIII metal and molybdenum compounds, phosphoric acid, as well as with stabilizers such as hydrogen peroxide and citric acid (monohydrate), when employed. It is preferred that the catalyst be impregnated by filling 95-105%, for example, 97% of the support pore volume with the stabilized impregnating solution containing the required amount of metals and phosphorus.

Finally, the impregnated support is oven-dried and then directly calcined preferably at 1000°-1150° F. for about 20 minutes to 2 hours in flowing air.

A hydroconversion process, such as a mild hydro-cracking process, which preferentially removes sulfur and nitrogen from the converted product stream with components having boiling points less than 1000° F. is desirable in those instances where there is less concern over the quality of the unconverted product stream, but, rather, where the primary concern is the quality of the distillate product from the hydroconversion process. It is well known to those skilled in the art that high heteroatom contents of distillate hydroconversion products have an adverse effect on fluid catalytic cracking of the heavier gas oils (having a boiling point of about 650° F. to about 1000° F.) and that extensive hydrotreating of the distillate streams would be required to meet the strict mandated levels of heteroatoms in distillate fuels. The demands placed upon catalyst compositions make it difficult to employ a single catalyst in a hydroconversion process, such as a mild hydro-cracking process, which will achieve effective levels of sulfur and nitrogen removal from the converted product stream having components with boiling points below 1000° F. However, the catalyst employed in the process of the instant invention is capable of achieving such results because the prescribed catalyst has an optimized micropore diameter to overcome the diffusion limitations for hydrotreatment of the converted product molecules but it also does not contain such large macropores that would allow poisoning of the catalyst pellet interior. The catalyst also has a very narrow pore size distribution such that pores with diameters less than 150 Angstroms are minimized as these pores are easily plugged with contaminants during hydroprocessing.

Catalyst Examples SN-6603, SN-6584, SN-6726 and SN-6785 the properties of which are described in Table III below, are catalysts prepared in the manner set out above, which may be employed in the MHC process of this invention. These catalysts were prepared with a support containing hydrogen form, acidified, dealuminated Y-zeolite obtained from American Cyanamid which is available in the form of extrudates in the diameter range of 0.035-0.041 inch.

TABLE III

#### NiMOP CATALYSTS ON SILICA-ALUMINA SUPPORTS CONTAINING HYDROGEN FORM, ACIDIFIED, DEALUMINATED Y-ZEOLITE

| Catalyst                                                                       | SN-6603 | SN-6584 | SN-6726 | SN-6785 |
|--------------------------------------------------------------------------------|---------|---------|---------|---------|
| Impreg. Sol'n.                                                                 | Ni—Mo—P | Ni—Mo   | Ni—Mo—P | Ni—Mo—P |
| SiO <sub>2</sub> , wt. %*                                                      | 2.0     | 2.0     | 0       | 0       |
| P <sub>2</sub> O <sub>5</sub> , wt. %                                          | 1.6     | 0       | 1.4     | 1.30    |
| MoO <sub>3</sub> , wt. %                                                       | 15.2    | 15.1    | 15.2    | 14.8    |
| NiO, wt. %                                                                     | 2.9     | 3.2     | 2.9     | 2.7     |
| Pore Volume Distribution by Hg Porosimetry: Surface Area by N <sub>2</sub> BET |         |         |         |         |
| Total PV, cc/g                                                                 | 0.68    | 0.72    | 0.61    | 0.60    |
| PV > 150Å, TPV                                                                 | 7.4     | 5.5     | 1.6     | 3.3     |
| PV > 250Å, TPV                                                                 | 25.0    | 25.0    | 19.7    | 33.3    |
| PV > 160Å, TPV                                                                 | 29.4    | 33.3    | 27.9    | 43.3    |
| PV < 160Å, TPV                                                                 | 64.7    | 66.7    | 70.5    | 58.3    |

TABLE III-continued

| NiMoP CATALYSTS ON SILICA-ALUMINA SUPPORTS CONTAINING HYDROGEN FORM, ACIDIFIED, DEALUMINATED Y-ZEOLITE |         |         |         |         |
|--------------------------------------------------------------------------------------------------------|---------|---------|---------|---------|
|                                                                                                        | SN-6603 | SN-6584 | SN-6726 | SN-6785 |
| PV < 100Å, TPV                                                                                         | 32.4    | 37.5    | 27.9    | 43.3    |
| PV 100-160Å, TPV                                                                                       | 33.0    | 29.2    | 42.6    | 28.3    |
| PV in PM $\pm$ 20A, % TPV                                                                              | 45.1    | 45.1    | 47.5    | 39.2    |
| PM at (dv/dD) max Å                                                                                    | 97      | 89      | 100     | 93      |
| PM (BET) Å                                                                                             | 89      | 89      | 90      | 87      |
| Surf. Area, m <sup>2</sup> /g                                                                          | 278     | 286     | 265     | 246     |
| HDS-MAT, C <sub>0.5g</sub> %                                                                           | 88      | 78      | 74      | 73      |
| <u>Zeolite</u>                                                                                         |         |         |         |         |
| Zeolite Content, wt. %                                                                                 | 16      | 15      | 16      | 26      |
| Zeolite Type**                                                                                         | ADAY    | ADAY    | ADAY    | ADAY    |
| UCS, Angstroms                                                                                         | 24.28   | 24.27   | 24.29   | 24.28   |
| SiO <sub>2</sub> /Al <sub>2</sub> O <sub>3</sub> ratio                                                 | 36      | 40      | 31      | 36      |
| <u>Metals Distribution by XPS Analysis</u>                                                             |         |         |         |         |
| Mo Gradient                                                                                            | 1.1     | 18.8    | 1.8     | 1.3     |
| Ni Gradient                                                                                            | 0.94    | 3.4     | 1.5     | 1.6     |
| (Mo/Al) <sub>int</sub>                                                                                 | 0.16    | 0.10    | 0.13    | 0.15    |
| MNi/Al) <sub>int</sub>                                                                                 | 0.018   | 0.015   | 0.014   | 0.015   |

\*The silica value in Table II is based on the wt. % of silica in the support.

\*\*ADAY - Hydrogen form, acidified, dealuminated Y-zeolite.

The properties of commercially available hydroprocessing catalyst A are set forth in Table IV below. Catalyst A is an available state of the art catalyst sold for use in hydroprocessing resid oils. Catalyst A, which is American Cyanamid HDS-1443B catalyst, is referred to in this specification as the standard reference catalyst.

Pore structure values set out in Tables III and IV were determined using Micrometrics Autopore 9220 Mercury Porosimetry Instrument.

TABLE IV  
ALUMINA BASED CATALYST AS CONTROL EXAMPLE

| Catalyst                                                                       | A         |
|--------------------------------------------------------------------------------|-----------|
| Impreg. Sol'n.                                                                 | Ni—Mo     |
| MoO <sub>3</sub> wt. %                                                         | 11.5-14.5 |
| NiO wt. %                                                                      | 3.2-4.0   |
| Pore Volume Distribution by Hg Porosimetry, Surface Area by N <sub>2</sub> BET |           |
| Total PV, cc/g                                                                 | 0.74      |
| PV > 250A, % TPV                                                               | 33.8      |
| PV > 160A, % TPV                                                               | 37.8      |
| PV < 160A, % TPV                                                               | 62.2      |
| PV < 100A, % TPV                                                               | 58.1      |
| PV 100-160A, % TPV                                                             | 4.1       |
| PM at (dv/dD) max Å                                                            | 50        |
| PM (BET), Å                                                                    | 46        |
| Surf. Area, m <sup>2</sup> /g                                                  | 314       |
| HDS-MAT, C <sub>0.5g</sub> %                                                   | 73        |
| <u>Metals Distribution by XPS Analysis</u>                                     |           |
| (Mo/Al) <sub>int</sub>                                                         | 0.09      |
| (Ni/Al) <sub>int</sub>                                                         | 0.012     |
| Mo Gradient                                                                    | 1.2       |
| Ni Gradient                                                                    | 1.6       |

A preferred feature of the catalyst composition of the instant invention is that the above-described oxide of molybdenum, preferably MoO<sub>3</sub>, is distributed on the above-described porous alumina support in such a manner that the molybdenum gradient of the catalyst has a value of about 1.0 to about 20.0, preferably about 1 to about 5. As used in this description and in the appended claims, the phrase "molybdenum gradient" means that the ratio of a given catalyst pellet exterior molybdenum/aluminum atomic ratio to a given catalyst pellet interior molybdenum/aluminum atomic ratio has a value of less than 6.0, preferably 1.0-5.0 the atomic ratios being measured by X-ray photoelectron spectroscopy (XPS), sometimes referred to as Electron Spectroscopy for Chemical Analysis (ESCA). It is theorized that the molybdenum gradient is strongly affected by the im-

pregnation of molybdenum on the catalyst support and the subsequent drying of the catalyst during its preparation. ESCA data on both catalyst pellet exteriors and interiors were obtained on an ESCALAB MKII instrument available from V. G. Scientific Ltd., which uses a 1253.6 electron volt magnesium X-ray source. Atomic percentage values were calculated from the peak areas of the molybdenum 3p<sub>3/2</sub> and aluminum 2p<sub>3/2</sub> signals using the sensitivity factors supplied by V. G. Scientific Ltd. The value of 74.7 electron volts for aluminum was used as a reference binding energy.

To determine the molybdenum/aluminum atomic ratio of a given catalyst pellet exterior for the catalyst of the instant invention, the catalyst pellets were stacked flat on a sample holder, and subjected to ESCA analysis. For the catalyst of the instant invention the molybdenum/aluminum atomic ratio of the catalyst pellet exterior is in the range of 0.12-2.0, preferably 0.15-0.75. This exterior molybdenum/aluminum atomic ratio is considerably greater than the Mo/Al catalyst surface atomic ratio of 0.03-0.09 disclosed in U.S. Pat. No. 4,670,132.

To determine the molybdenum/aluminum atomic ratio of a given catalyst pellet interior for the catalyst of the instant invention, the catalyst pellets were crushed into a powder, placed firmly in a sample holder, and subjected to ESCA analysis. For the catalyst of the instant invention, the molybdenum/aluminum atomic ratio of the catalyst pellet interior (i.e., the molybdenum/aluminum ratio of the powder, which is assumed to be representative of the interior portion of the pellet) is in the range of 0.10-0.20, preferably 0.11-0.18.

The molybdenum/aluminum atomic ratios of the total catalyst composition of the instant invention, as determined by conventional means (i.e., Atomic Absorption (AA) or Inductively Coupled Plasma (ICP) spectroscopies) is in the range of 0.060-0.075, preferably 0.062-0.071. To determine the total catalyst composition molybdenum/aluminum atomic ratio, catalyst pellets were ground to a powder and digested in acid to form an ionic solution. The solution was then measured by AA or ICP to determine Mo ion concentration, which was then adjusted to MoO<sub>3</sub> concentration. Alumina (Al<sub>2</sub>O<sub>3</sub>) concentration was back-calculated from the direct measurement of the concentration of the other components (e.g., Ni, Fe, Na, S).

The HDS Microactivity Test (HDS-MAT) was used to evaluate the intrinsic activity of catalysts in the absence of diffusion and using a model sulfur compound as a probe. The catalyst, ground to a 30-60 mesh fraction, is presulfided at 750 F. with a 10% H<sub>2</sub>S/H<sub>2</sub> mixture for 2 hours. The presulfided catalyst is exposed to a benzothiophene-containing feed at 550° F. and flowing hydrogen for approximately four hours. Cuts are taken periodically and analyzed by a gas chromatograph for the conversion of benzothiophene to ethylbenzene. The results obtained with HDS-MAT tests as well as the Mo and Ni gradients of the catalysts described are shown in Tables III and IV.

#### BERTY REACTOR HYDROCRACKING CATALYST EVALUATION

The Berty reactor, a type of continuous stirred tank reactor (CSTR), was used to determine hydrocracking activities of the catalysts of this invention in a diffusion controlled regime at a low rate of deactivation. The catalysts were presulfided and then the reaction was carried out at a single space velocity for 38 hours. The sample cuts were taken every 4 hours and tested for boiling point distribution, is Ni, V, S, and sediment content. Using these data, conversions for the 650° F. + and 1000° F. + fractions were determined. The feedstock properties and the operating conditions of the Berty reactor are listed in Table V which follows.

TABLE V

| BERTY REACTOR OPERATING CONDITION |                                                                                                                                                                 |
|-----------------------------------|-----------------------------------------------------------------------------------------------------------------------------------------------------------------|
| <u>1. PRESULFIDING</u>            |                                                                                                                                                                 |
| Temperature                       | 750°-800° F.                                                                                                                                                    |
| Pressure                          | 40 Psig                                                                                                                                                         |
| Gas Mixture                       | 10 Vol % H <sub>2</sub> S - 90 Vol % H <sub>2</sub>                                                                                                             |
| Gas Flow                          | 500 SCCM                                                                                                                                                        |
| Duration                          | 2 Hr., 45 Min.                                                                                                                                                  |
| <u>2. FEEDSTOCK</u>               |                                                                                                                                                                 |
| Boiling Point Distribution        | 60 Vol % Desulfurized VGO<br>40 Vol % Ar M/H Vac. Resid<br>IBP 444° F.<br>PPB 1371° F.<br>650° F. + 89.2 Vol %<br>900° F. + 45.6 Vol %<br>1000° F. + 33.5 Vol % |
| Sulfur wt %                       | 2.2                                                                                                                                                             |
| Ni Content, ppm                   | 20                                                                                                                                                              |
| V Content, ppm                    | 54                                                                                                                                                              |
| <u>3. REACTION CONDITIONS</u>     |                                                                                                                                                                 |
| Temperature                       | 805° F.                                                                                                                                                         |
| Pressure                          | 1000 Psig                                                                                                                                                       |
| Hydrogen Feed Rate                | 300 SCCM                                                                                                                                                        |
| Liquid Feed Rate                  | 82.5 CC/Hr                                                                                                                                                      |
| Liquid Holdup                     | 125 CC                                                                                                                                                          |
| Catalyst Charge                   | 36.9 Grams                                                                                                                                                      |

The hydrocracking activity was determined by comparing the percentages of products in the 650° F. - fraction and 1000° F. - fraction when various catalysts were evaluated under constant mild hydrocracking conditions with the same feedstock. The conversions of 650° F. + and 1000° F. + were calculated by the equations below:

$$\text{Conversion} = \frac{Y(F) - Y(P)}{Y(F)} \times 100\%$$

Y(F) denotes the volume percentage of the 650° F. + or 1000° F. + fraction in the feedstock.

Y(P) denotes the volume percentage of the 650° F. + or 1000° F. + fraction in the products.

-continued

The boiling point distribution of the total product was determined using the ASTM D-2887 Method, Simulated Distillation by Gas Chromatography. The existent sediment content in the total product was measured by using the IP 375/86 Method, Total Sediment in Residual Fuels. The Total Sediment is the sum of the insoluble organic and inorganic material which is separated from the bulk of the residual fuel oil by filtration through a filter medium, and which is also insoluble in a predominantly paraffinic solvent.

Data listed in Table VI, which follows, show the activity results achieved with Catalyst SN-6584 and SN-6603 which are catalysts of this invention compared to the activities exhibited by Catalyst A (the reference catalyst) and Catalyst B, which are commercially available hydroprocessing catalysts, as determined in the Berty Reactor tests.

The data of Table VI show that Catalyst SN-6603 exhibits a 650° F. + conversion value substantially greater than Catalyst A and greater than Catalyst B; a 1000° F. + conversion value substantially greater than Catalyst A and greater than Catalyst B; a sediment value substantially lower than Catalyst B and somewhat less than Catalyst A and Catalyst SN-6603 exhibits an HDS activity substantially greater than Catalysts A and B, both of which are commercial hydroprocessing catalysts.

With regard to Catalyst SN-6584, the data presented in Table VI show that Catalyst SN-6584 exhibits a 650° F. + conversion value substantially greater than Catalyst A and somewhat less than Catalyst B; a 1000° F. + conversion value greater than Catalyst A and somewhat lower than Catalyst B; a sediment value somewhat less than Catalyst A and significantly less than Catalyst B and an HDS activity greater than Catalyst A and substantially greater than Catalyst B.

TABLE VI

| Catalyst | BERTY RESID MILD HYDROCRACKING ACTIVITIES TEMPERATURE TEST RESULTS |                                   |                     |                      |
|----------|--------------------------------------------------------------------|-----------------------------------|---------------------|----------------------|
|          | 650° F. +<br>Conversion<br>Vol %                                   | 1000° F. +<br>Conversion<br>Vol % | IP<br>Sediment<br>% | HDS<br>Activity<br>% |
| A        | 29                                                                 | 78                                | 0.7                 | 69                   |
| B        | 47                                                                 | 86                                | 1.0                 | 63                   |
| *SN-6603 | 49                                                                 | 90                                | 0.6                 | 76                   |
| *SN-6584 | 42                                                                 | 83                                | 0.6                 | 71                   |

Run conditions: Temperature = 805° F., Pressure = 1000 Psig, LHSV = 0.66, Hydrogen Flow Rate = 300 SCCM, and the feedstock is 40 Vol % Arabian Medium/Arabian Heavy (65:35 Vol %) vacuum resid in desulfurized vacuum gas oil.

\*Catalyst of the instant invention.

A comparison of the conversion advantages of Catalysts SN-6603 and SN-6584 as compared to conversion and sediment values for commercial hydroprocessing Catalysts A and B is set out in the data presented in Table VII which follows.

TABLE VII

| Catalyst | Catalyst<br>Type | BERTY RESID MILD HYDROCRACKING ACTIVITIES Test Results Compared to Results with Standard Catalyst A |                                                |                              |  |
|----------|------------------|-----------------------------------------------------------------------------------------------------|------------------------------------------------|------------------------------|--|
|          |                  | 650° F. +<br>Conversion<br>Advantage<br>Vol %                                                       | 1000° F. +<br>Conversion<br>Advantage<br>Vol % | IP<br>Sediment<br>Delta<br>% |  |
| A        | Alumina          | 0                                                                                                   | 0                                              | 0                            |  |
| B        | Zeolite/         | +18                                                                                                 | +8                                             | +0.3                         |  |

TABLE VII-continued

| BERTY RESID MILD HYDROCRACKING ACTIVITIES                 |               |                                      |                                       |                     |    |
|-----------------------------------------------------------|---------------|--------------------------------------|---------------------------------------|---------------------|----|
| Test Results Compared to Results with Standard Catalyst A |               |                                      |                                       |                     |    |
| Catalyst                                                  | Catalyst Type | 650° F. + Conversion Advantage Vol % | 1000° F. + Conversion Advantage Vol % | IP Sediment Delta % |    |
| *SN-6603                                                  | Alumina       |                                      |                                       |                     |    |
| *SN-6603                                                  | ADAY-Silica   | +20                                  | +12                                   | -0.1                | 5  |
| *SN-6584                                                  | Alumina       |                                      |                                       |                     | 10 |
| *SN-6584                                                  | ADAY-Silica   | +13                                  | +5                                    | -0.1                | 15 |
|                                                           | Alumina       |                                      |                                       |                     | 20 |

Run conditions: Temperature = 805° F., Pressure = 1000 Psig, LHSV = 0.66, Hydrogen Flow Rate = 300 SCC/M, and the feedstock is 40 Vol % Arabian Medium/Arabian Heavy (65:35 Vol %) vacuum resid in desulfurized vacuum gas oil.

\*Catalysts of the instant invention.

\*ADAY - Hydrogen form, acidified, dealuminated Y-zeolite.

The data presented in Table VII show that Catalyst SN-6603, a catalyst of the instant invention, exhibits an increase of 20 Vol % in 650° F. conversion or about a 69% improvement in relative conversion over that achieved with Catalyst A (i.e., the standard base commercial catalyst). Catalyst SN-6603 also gave an appreciable improvement in the 1000° F. + conversion (12 Vol %) or about a 15% improvement in relative conversion over that achieved with Catalyst A. The IP sediment make for Catalyst SN-6603 showed a small decrease over the sediment make of Catalyst A and a substantial decrease in the sediment make of Catalyst B.

With regard to Catalyst SN-6584 the data in Table VII show that an increase of 13 Vol % in the 650° F. + conversion value (i.e., about a 45% improvement in relative conversion over that achieved with Catalyst A) and in the 1000° F. + conversion value Catalyst SN-6584 gave a 5 Vol % improvement or 6.4% in relative conversion over Catalyst A while the IP sediment value decreased 0.1% over Catalyst A.

The high sediment make of Catalyst B, as the data in Tables VI and VII show, indicates that this catalyst would not be suitable for use in the MHC process of this invention because of a distinct tendency to cause reactor plugging.

The results set out in Table VII clearly indicate that Catalysts SN-6603 and SN-6584, the zeolite containing catalysts of the invention, substantially outperforms Catalysts A and B of the prior art.

Mild hydrocracking of heavy oils containing resids in the presence of the catalyst of this invention comprising, for example, molybdenum oxide, nickel oxide, and, optionally, phosphorus oxide on the zeolite-containing alumina support having a specified pore size distribution not only allows an increased production of middle distillate and more effective conversion of resid feedstocks but also maintains the sediment make at a low level similar to or lower than that achieved with conventional bimodal alumina based catalysts.

What is claimed is:

1. A process for mild hydrocracking of a hydrocarbon feedstock having a substantial proportion of com-

ponents boiling below about 1000° F., said process comprising contacting said hydrocarbon feedstock under conditions of elevated temperature and a hydrogen pressure of less than about 1500 psig with a particulate catalyst comprising about 1.0 to about 6.0 wt. % of an oxide of a Group VIII metal; about 12.0 to about 25.0 wt. % of an oxide of molybdenum and 0.1 to about 3.0 wt. % of an oxide of phosphorus all supported on a porous support comprising (1) a matrix selected from the group consisting of precipitated alumina and silica-alumina containing about 1.0 to about 3.0 wt. % of silica and (2) about 5.0 to about 35 wt. %, based on the weight of the support, of hydrogen form, acidified, dealuminated Y-zeolite having a silica to alumina mole ratio of about 10-120, a secondary pore volume of about 0.14-0.20 cc/g, a unit cell size of about 24.23-24.33 Å, a secondary pore mode of about 115-145 Å, a secondary pore diameter of about 100-600 Å, a surface silicon to aluminum atom ratio of about 24-45, and an acid site density of about 1-5 cc NH<sub>3</sub>/g of zeolite, in such a manner that the molybdenum gradient of the catalyst ranges from about 1 to about 20, said conditions being such as to yield about a 10 to about a 60 Vol % conversion of the hydrocarbon feedstock boiling above 650° F. to hydrocarbon products boiling at or below 650° F., wherein the said catalyst is characterized by having about 40 to about 65% of the total pore volume in pores of diameters from about 20 Å below the pore mode diameter to about 20 Å above the pore mode diameter and the pore mode diameter is in the range of about 80 to about 120 Å and wherein the said catalyst is further characterized by having a total surface area of about 200 to about 300 m<sup>2</sup>/g and a total pore volume of about 0.55 to about 0.75 cc/g, with a pore volume distribution such that micropores having diameters less than 100 Å constitute less than 40%, pores having diameters of 100-160 Å constitute about 25 to about 50%, pores having diameters greater than 160 Å constitute about 25 to about 50% of the total pore volume of the catalyst, macropores having diameters greater than 250 Å constitute about 15 to about 40%, and macropores having diameters greater than 1500 Å constitute less than 10% of the total pore volume.

2. The process of claim 1 wherein the said hydrocarbon feedstock is contacted with said catalyst in a fixed bed reactor.

3. The process of claim 1 wherein the said hydrocarbon feedstock is contacted with said catalyst in a single ebullated bed reactor.

4. The process of claim 1 wherein the said hydrocarbon feed is contacted with said catalyst in a series of 2-5 ebullated bed reactors.

5. The process of claim 1 wherein the said hydrocarbon feed is contacted with said catalyst in a series of 2-5 continuous stirred tank reactors.

6. The process of claim 1 wherein the said hydrocarbon feed is contacted with said catalyst in a single continuous stirred tank reactor.

\* \* \* \* \*